

Aug. 17, 1954

W. J. COOK ET AL

2,686,757

SUPPRESSION OF HONEYCOMBING IN CATHODE NICKEL

Filed Jan. 15, 1953

*HONEYCOMBED NICKEL CATHODE*



*Fig. 1.*

*SOUND NICKEL CATHODE*



*Fig. 2.*

INVENTORS  
WILFRED JAMES COOK  
WILBUR VERNON BARKER  
JOSEPH HOWARD TUCK

BY *G. Jr. Miller*  
ATTORNEY

## UNITED STATES PATENT OFFICE

2,686,757

SUPPRESSION OF HONEYCOMBING IN  
CATHODE NICKEL

Wilfred James Cook, Wilbur Vernon Barker, and  
Joseph Howard Tuck, Port Colborne, Ontario,  
Canada, assignors to The International Nickel  
Company, Inc., New York, N. Y., a corporation  
of Delaware

Application January 15, 1953, Serial No. 331,480

Claims priority, application Canada  
November 21, 1952

16 Claims. (Cl. 204—113)

1

The present invention relates to improved electrorefining of nickel and, more particularly, to a process for producing sound cathode nickel and to an electrolyte for use in said process.

For many years, the art of electrorefining nickel was confronted with the problem of "honeycombing." In some instances, the problem was more serious than in others. Many different factors, such as process variables, construction materials, electrolyte composition variables, etc., were scrutinized in a search for the cause of "honeycombing" but this scrutiny revealed neither the cause of nor a solution to this problem. Efforts to solve the problem of "honeycombing" by making a large number of changes and variations in the process, the apparatus, the electrolyte composition, the treatment of the mother blanks used in producing the starting sheets, etc., were not fully acceptable as a wholly successful solution on a commercial scale to the problem of "honeycombing." Thus, the addition of cobalt into the electrolyte, for example, as cobalt chloride, was not effective in suppressing "honeycombing." Likewise, using other means, such as nickel peroxide for precipitating cobalt, was not satisfactory. Changing the materials of which the apparatus was composed, for example, replacing the cotton on the cathode boxes with synthetic fibers, replacing the pine side sticks on the electrolytic cell with cypress or protecting the side sticks with various materials, did not solve the problem. The addition of various addition agents to the correction tank, for example, cuprous chloride, sodium hypochlorite, sulfur dioxide, hydrogen peroxide and combinations thereof, also was unsuccessful. Adding to the cathode boxes or compartments various chemicals, such as sodium chlorate, sodium perborate, potassium permanganate, manganous sulfate, cobalt chloride, cupric sulfate, ferrous sulfate, boric acid, quebracho, bindarine, or the boiled extract of cypress chips, also did not solve the problem. Certain expedients, such as adding hydrogen peroxide to combine with hydrogen, vibrating the cathodes, and bubbling finely dispersed air through the catholyte through a porous tube beneath the cathode, were not successful in overcoming "honeycombing," although such expedients usually overcome pitting which is a different condition generally attributed by those skilled in the art to be due to the adherence of cathodically evolved hydrogen. Other unacceptable expedients which were tried include (1) varying the process conditions, for example, decreasing the current density, operating the process at various

2

reduced pH values, boiling the purified electrolyte under vacuum or varying the rate of flow of the electrolyte; (2) modifying the process, for example, by triple pressing through an oxidizing slime while adding oxidizing agents, such as chlorine, hydrogen peroxide or sodium hypochlorite, ahead of the filter press; and (3) pretreating the stainless steel mother blanks upon which the cathode nickel starting sheets are electrodeposited with various agents, for example, nitric acid, hydrofluoric acid, etc. Although these and many other attempts were made to overcome the foregoing difficulties and to solve the problem of honeycombing, none was entirely successful when carried into practice commercially on an industrial scale.

It has now been discovered that improved, sound, pure nickel cathodes substantially free from honeycombing can be produced in an electrorefining operation in an improved and efficient manner, utilizing the sulfate-chloride electrolyte process, by the addition of critical amounts of special organic compounds to the purified electrolyte.

25 It is an object of the present invention to provide an improved process for producing sound nickel cathodes substantially free from honeycombing.

Another object of the invention is to provide 30 an improved bath from which nickel cathodes, substantially free from honeycombing, may be deposited by electrolysis.

Still another object of the invention is to provide 35 a method for suppressing or eliminating honeycombing in electrorefined cathode nickel.

It is a further object of the invention to provide 40 an improved nickel electrorefining process for the production of sound nickel cathodes substantially free from honeycombing while utilizing the sulfate-chloride electrolyte.

Other objects and advantages will become apparent from the following description taken in conjunction with the accompanying drawings, in which:

Figure 1 is a reproduction of a photomicrograph at 1 diameter of a cross section of a honeycombed nickel cathode; and

Figure 2 is a reproduction of a photomicrograph at 1 diameter of a cross section of a sound nickel cathode produced in accordance with the present invention.

Generally speaking, the present invention contemplates a process for the production of commercially acceptable cathode nickel substantially free from the deleterious effects of honeycombing

which comprises electrolyzing an aqueous electrolyte having a pH between about 3.0 and about 5.0 and containing about 40 to about 70 g. p. l. (grams per liter) of nickel, about 12 to about 30 g. p. l. of sodium, about 18 to about 55 g. p. l. of chloride radical, about 65 to about 115 g. p. l. of sulfate radical, about 15 to about 25 g. p. l. of boric acid and about 0.0003 to about 0.001 g. p. l. of at least one terminally substituted polyethylene oxide condensate selected from the group consisting of a polyethylene oxide condensate of m-methyl p-octyl phenol containing 8 to 11 moles of ethylene oxide per mole and a polyethylene oxide condensate of lauryl alcohol containing 4 to 6 moles of ethylene oxide per mole to electrodeposit sound nickel at the cathode. The electrolysis is carried out while maintaining the electrolyte temperature between about 100° F. and about 160° F. and while employing a current density up to between about 5 and about 25 amperes per square foot. The catholyte may contain a total of up to about 0.004 g. p. l. of such impurities as copper, iron, arsenic, lead, etc., without affecting the operating characteristics of the process. In addition, the catholyte may be saturated with respect to calcium ions. Thus, it may contain up to about 0.6 g. p. l. of calcium, without affecting the operating characteristics of said process. The process utilizing the aforementioned electrolyte is applicable not only to the production of commercial cathode nickel but also to the production on mother blanks of the thin nickel cathode starting sheets employed in producing commercial cathode nickel.

The aforementioned terminally substituted polyethylene oxide condensates, a polyethylene oxide condensate of m-methyl p-octyl phenol containing 8 to 11 moles of ethylene oxide per mole and a polyethylene oxide condensate of lauryl alcohol containing 4 to 6 moles of ethylene oxide per mole, which are utilized as honeycomb-suppressing agents in carrying out the present invention, may be represented by their respective structural formulas as follows:



and

where  $n$  is 4 to 6

If more than 0.001 g. p. l., for example 0.005 g. p. l., of said compounds is present in the catholyte, the production of the cathode nickel is detrimentally affected due to the fact that the resultant cathodes becomes highly stressed and/or warped. Stresses set up in the nickel deposited on the stainless steel mother blanks to form the cathode starting sheets and due to excessive amounts of the aforementioned compounds are often so great that the cathode nickel separates from the mother blanks and the resulting starting sheets are badly warped. Attempts to straighten these warped starting sheets are defeated by their "springy" reaction due to the high stresses. The production of the commercial cathode nickel is also adversely affected when excessive amounts of the additives are employed in that the cathodes become highly stressed and warped and difficulty is encountered in extricating these warped cathodes from the cathode boxes and in thereafter straightening them. When less than about 0.0003 g. p. l., for example, 0.0001 g. p. l., of said

compounds is present in the catholyte, there is no substantial suppression of honeycombing. It has been found that other compounds, similar in certain respects to the honeycomb suppressors contemplated for use in practicing applicants' invention, are inoperative in preventing honeycombing in concentrations sufficiently low to avoid the production of undesirably stressed nickel cathodes. Such inoperative compounds include a polyethylene oxide condensate of nonyl phenol represented as follows:



15

The addition of the special compounds in the aforementioned critical amounts contemplated by the present invention has not been found to have any demonstrable effect upon the characteristics and properties of the electrolyte, other than that of substantially suppressing honeycombing. For example, no substantial decrease is found in the surface tension of the electrolyte. Thus, the surface tension of the electrolyte, as measured with a Cenco Du Nouy tensiometer, prior to the introduction of the honeycomb-suppressing agent contemplated by the present invention is usually about 76 to about 78 dynes per centimeter when measured at 25° C.; and the surface tension of the electrolyte after introduction of the aforementioned honeycomb-suppressing agents in amounts contemplated by this invention is usually about 70 to about 78 dynes per centimeter when measured at 25° C., which compares with 72 dynes per centimeter as the surface tension of water determines under similar conditions. However, if excessive amounts of one of these compounds are added, such as about 0.01 g. p. l., the surface tension is radically lowered to about 35 to 40 dynes per centimeter which is indicative of a marked change in the characteristics and properties of the electrolyte and may have some relation to the fact that cathode nickel produced from such an electrolyte is unsatisfactory.

45

In carrying the invention into practice to produce cathode nickel, it is preferred to electrolyze an aqueous catholyte having a pH about 3.8 to 4.6 and containing about 40 to about 60 g. p. l. of nickel, about 18 to about 30 g. p. l. of sodium, about 65 to about 99 g. p. l. of sulfate radical, about 27 to about 51 g. p. l. of chloride radical, about 15 to about 25 g. p. l. of boric acid, about 0.0004 to about 0.0008 g. p. l. of the aforementioned honeycomb-suppressing agent, and the balance essentially water to electrodeposit nickel at the cathode. The electrolysis is carried out by passing electric current through an anode (in practice, usually impure nickel), the electrolyte and the cathode (usually a nickel starting sheet) while maintaining the temperature between about 130° F. and about 150° F. and while employing a current density between about 12 and about 20 amperes per square foot. Although an impure nickel anode containing about 90% to about 96% of nickel is employed, the process is also operative when utilizing insoluble anodes. When using soluble impure nickel anodes, the composition of the anode is dependent upon the source of nickel. Thus, for example, in one industrial operation, the impure nickel anodes contain about 94% to about 96% of nickel, about 2.5% to about 3.5% of copper, about 0.7% to about 0.9% of cobalt, about 0.5% to about 1.0% of iron, about 0.002% to about 0.004% of lead, about 0.05% to about 0.07% of arsenic and about 0.5% to about 0.8%

## 5

of sulfur. It is further preferred that the electrolyte be continuously circulated from the cells through a purification system and back to the cathodes to prevent depletion of the constituents.

The electrolyte may advantageously be prepared by the anodic dissolution of nickel in a solution of boric acid, sodium chloride and an amount of sulfuric acid equivalent to the desired nickel. However, the dissolution of nickel sulfate together with sodium chloride, boric acid and sodium carbonate for pH adjustment would be a preferred method of preparing electrolyte. Prior to the production of cathode nickel in accordance with the present invention, the electrolyte may be subjected to various treatments and operations known to the art to accomplish purposes, such as purification, conditioning, control, etc. For example, the electrolyte may be treated and/or processed prior to the production of cathode nickel and/or the introduction of the honeycomb-suppressing agent in accordance with the teaching of the Renzoni U. S. Patent No. 2,394,874. Likewise, after the production of the cathode nickel, the depleted or spent electrolyte may be subjected to further treatment and/or processing to replenish the nickel content and to accomplish other objectives such as purification, conditioning, adjustment of composition, control, etc. Furthermore, the process contemplated by the present invention may be carried out in any type of suitable electrolytic apparatus, including that referred to and/or disclosed in the Renzoni U. S. Patents Nos. 2,394,874 and 2,480,771. Thus, in actual practice, an impure nickel anode may be anodically corroded by a sulfate-chloride acid anolyte in the anode compartment of a compartmented electrolytic cell. This impure anolyte is then purified in a separate purification circuit with the removal of copper, iron, arsenic, and lead. The now-purified electrolyte is finally introduced into the cathode compartment of the aforementioned cell and electrolyzed to electrodeposit nickel on the cathode starting sheet.

For the purpose of giving those skilled in the art a better understanding of the invention and a better appreciation of the advantages of the invention, the following illustrative examples are given:

*Example I*

To a portion of an electrolyte which, after treatment with chlorine to remove cobalt, was found to result in the production of honeycombed cathode nickel, about 0.0005 g. p. l. of polyethylene oxide condensate of m-methyl p-octyl phenol containing 8 to 11 moles of ethylene oxide per mole was added. The electrolyte was not otherwise modified in composition. The electrolyte, after the addition of the aforementioned amounts of honeycomb-suppressing agent, had a pH of 4.0 and contained 52 g. p. l. of nickel, 22 g. p. l. of sodium, 40 g. p. l. of chloride radical, 78 g. p. l. of sulfate radical, 15 g. p. l. of boric acid, 0.0005 g. p. l. of a polyethylene oxide condensate of m-methyl, p-octyl phenol containing 8 to 11 moles of ethylene oxide per mole and the balance essentially water. The surface tension of this electrolyte, as measured by a Cenco Du Nouy Tensiometer at 25° C., was about 75 dynes per centimeter. The aforementioned electrolyte containing the honeycomb-suppressing agent was electrolyzed to electrodeposit cathode nickel at the same current density and temperature, i. e., 15 amperes per square foot and 140° F., as had initially produced honeycombed nickel. The resulting cathode

## 6

nickel produced therefrom was found to be substantially stress free and unwarped and devoid of honeycombing. Upon macrographic examination the cathode nickel thus produced was found to have a sound structure similar to that shown in Figure 2.

*Example II*

To another portion of the same electrolyte which, after treatment with chlorine to remove cobalt, was found to result in the production of honeycombed cathode nickel, about 0.0008 g. p. l. of a polyethylene oxide condensate of lauryl alcohol containing 4 moles of ethylene oxide per mole was added. The electrolyte was not otherwise modified in composition. The electrolyte, after the addition of the aforementioned amounts of honeycomb-suppressing agent, had a pH of 4.0 and contained 50 g. p. l. of nickel, 20 g. p. l. of sodium, 40 g. p. l. of chloride radical, 70 g. p. l. of sulfate radical, 6 g. p. l. of boric acid, 0.0008 g. p. l. of a polyethylene oxide condensate of lauryl alcohol containing 4 moles of ethylene oxide per mole and the balance essentially water. The surface tension of this electrolyte, as measured by a Cenco Du Nouy tensiometer, was about 72 dynes per centimeter. The aforementioned electrolyte containing the honeycomb-suppression agent was electrolyzed to electro-deposit cathode nickel at the same current density and temperature, i. e., 15 amperes per square foot and 140° F., as had initially produced honeycombed nickel. The resulting cathode nickel produced therefrom was found to be substantially stress free and unwarped and devoid of honeycombing. Upon macrographic examination the cathode nickel thus produced was found to have a sound structure similar to that shown in Figure 2.

*Example III*

To still another portion of the same electrolyte which, after treatment with chlorine to remove cobalt, was found to result in the production of honeycombed cathode nickel, about 0.00045 g. p. l. of a polyethylene oxide condensate of lauryl alcohol containing 6 moles of ethylene oxide per mole was added. The electrolyte was not otherwise modified in composition. The electrolyte, after the addition of the aforementioned amounts of honeycomb-suppressing agent, had a pH of 4.0 and contained 56 g. p. l. of nickel, 26 g. p. l. of sodium, 44 g. p. l. of chloride radical, 89 g. p. l. of sulfate radical, 17 g. p. l. of boric acid, 0.00045 g. p. l. of a polyethylene oxide condensate of lauryl alcohol containing 6 moles of ethylene oxide per mole and the balance essentially water. The surface tension of this electrolyte, as measured at 25° C. by a Senco Du Nouy tensiometer, was about 75 dynes per centimeter. The aforementioned electrolyte containing the honeycomb-suppressing agent was electrolyzed to electrodeposit cathode nickel at the same current density and temperature, i. e., 15 amperes per square foot and 140° F., as had initially produced honeycombed nickel. The resulting cathode nickel produced therefrom was found to be substantially stress free and unwarped and devoid of honeycombing. Upon macrographic examination the cathode nickel thus produced was found to have a sound structure similar to that shown in Figure 2.

While the invention has been described with particular emphasis upon an electrolyte containing the honeycomb-suppression agents described hereinbefore, it is to be noted that another aspect of the invention resides in an electrorefining proc-

ess utilizing applicants' particular bath composition and operating conditions. Likewise, while particular emphasis has been placed upon the presence of the aforementioned honeycomb-suppressing agents in critical amounts in the electrolyte, it is not to be intended to imply that the remaining composition of electrolyte is unimportant. On the contrary, the presence of chloride radical in the electrolyte is an important aspect of the invention since honeycombing has not been observed to occur when the electrolyte is an all-sulfate electrolyte devoid of chloride radical or is an electrolyte low in chloride radical. The invention is applicable in its broader aspects to the production of cathode nickel from any high chloride electrolyte having a composition within the ranges set forth hereinbefore where it is desired to insure the suppression of honeycombing in cathode nickel.

Although the present invention has been described in conjunction with preferred embodiments, it is to be understood that modifications and variations may be resorted to without departing from the spirit and scope of the invention, as those skilled in the art will readily understand. Thus, for the purposes of this invention cobalt is the equivalent of nickel. Such modifications and variations are considered to be within the purview and scope of the invention and appended claims.

We claim:

1. A process for the electrorefining of nickel from an aqueous nickel-containing solution which comprises establishing a catholyte having a pH between about 3 and about 5 comprising between about 40 to about 70 g. p. l. of nickel, about 12 to about 30 g. p. l. of sodium, about 18 to about 55 g. p. l. of chloride radical, about 65 to about 115 g. p. l. of sulfate radical, about 15 to about 25 g. p. l. of boric acid and about 0.0003 to about 0.001 g. p. l. of at least one compound selected from the group consisting of a compound having the structural formula



where  $m$  is 8 to 11 and a compound having the structural formula



where  $n$  is 4 to 6 with the balance essentially water, and electrolyzing said catholyte while maintaining the temperature between about 100° F. and about 160° F. by passing electric current at a current density between about 5 and about 25 amperes per square foot through said electrolyte from an anode to a cathode to deposit sound nickel cathodes.

2. A process for the electrorefining of nickel from an aqueous nickel-containing solution which comprises establishing a catholyte having a pH between about 3 and about 5 comprising between about 40 to about 70 g. p. l. of nickel, about 12 to about 30 g. p. l. of sodium, about 18 to about 55 g. p. l. of chloride radical, about 65 to about 115 g. p. l. of sulfate radical, about 15 to about 25 g. p. l. of boric acid and about 0.0003 to about 0.001 g. p. l. of a compound having the structural formula



Where  $m$  is 8 to 11

with the balance essentially water, and electrolyz-

ing said catholyte while maintaining the temperature between about 100° F. and about 160° F. by passing electric current at a current density between about 5 and about 25 amperes per square foot through said electrolyte from an anode to a cathode to deposit sound nickel cathodes.

3. A process for the electrorefining of nickel from an aqueous nickel-containing solution which comprises establishing a catholyte having a pH between about 3 and about 5 comprising between about 40 to about 70 g. p. l. of nickel, about 12 to about 30 g. p. l. of sodium, about 18 to about 55 g. p. l. of chloride radical, about 65 to about 115 g. p. l. of sulfate radical, about 15 to about 25 g. p. l. of boric acid and about 0.0003 to about 0.001 g. p. l. of a compound having the structural formula



with the balance essentially water, and electrolyzing said catholyte while maintaining the temperature between about 100° F. and about 160° F. by passing electric current at a current density between about 5 and about 25 amperes per square foot through said electrolyte from an anode to a cathode to deposit sound nickel cathodes.

4. A process for the electrorefining of nickel from an aqueous nickel-containing solution which comprises establishing a catholyte having a pH between about 3 and about 5 comprising between about 40 to about 70 g. p. l. of nickel, about 12 to about 30 g. p. l. of sodium, about 18 to about 55 g. p. l. of chloride radical, about 65 to about 115 g. p. l. of sulfate radical, about 15 to about 25 g. p. l. of boric acid and about 0.0003 to about 0.001 g. p. l. of a compound having the structural formula



40 with the balance essentially water, and electrolyzing said catholyte while maintaining the temperature between about 100° F. and about 160° F. by passing electric current at a current density between about 5 and about 25 amperes per square foot through said electrolyte from an anode to a cathode to deposit sound nickel cathodes.

5. A process for the electrorefining of nickel from an aqueous nickel-containing solution which comprises establishing a catholyte having a pH between about 3.8 and about 4.6 comprising between about 40 to about 60 g. p. l. of nickel, about 18 to about 30 g. p. l. of sodium, about 27 to about 51 g. p. l. of chloride radical, about 65 to about 99 g. p. l. of sulfate radical, about 15 to about 25 g. p. l. of boric acid and about 0.0004 to about 0.0008 g. p. l. of at least one terminally substituted polyethylene oxide condensate selected from the group consisting of a polyethylene oxide condensate of *m*-methyl *p*-octyl phenol containing 8 to 11 moles of ethylene oxide per mole and a polyethylene oxide condensate of lauryl alcohol containing 4 to 6 moles of ethylene oxide per mole with the balance essentially water, and electrolyzing said catholyte while maintaining the temperature between about 130° F. and about 150° F. by passing electric current at a current density between about 12 and about 25 amperes per square foot through said electrolyte from an anode to a cathode to deposit sound nickel cathodes.

6. A process for the electrorefining of nickel from an aqueous nickel-containing solution which comprises establishing a catholyte having a pH between about 3.8 and about 4.6 comprising between about 40 to about 60 g. p. l. of nickel, about

18 to about 30 g. p. l. of sodium, about 27 to about 51 g. p. l. of chloride radical, about 65 to about 99 g. p. l. of sulfate radical, about 15 to about 25 g. p. l. of boric acid and about 0.0004 to about 0.0008 g. p. l. of a compound having the structural formula



Where  $m$  is 8 to 11

with the balance essentially water, and electrolyzing said catholyte while maintaining the temperature between about 130° F. and about 150° F. by passing electric current at a current density between about 12 and about 25 amperes per square foot through said electrolyte from an anode to a cathode to deposit sound nickel cathodes.

7. A process for the electrorefining of nickel from an aqueous nickel-containing solution which comprises establishing a catholyte having a pH between about 3.8 and about 4.6 comprising between about 40 to about 60 g. p. l. of nickel, about 18 to about 30 g. p. l. of sodium, about 27 to about 51 g. p. l. of chloride radical, about 65 to about 99 g. p. l. of sulfate radical, about 15 to about 25 g. p. l. of boric acid and about 0.0004 to about 0.0008 g. p. l. of a compound having the structural formula



with the balance essentially water, and electrolyzing said catholyte while maintaining the temperature between about 130° F. and about 150° F. by passing electric current at a current density between about 12 and about 25 amperes per square foot through said electrolyte from an anode to a cathode to deposit sound nickel cathodes.

8. A process for the electrorefining of nickel from an aqueous nickel-containing solution which comprises establishing a catholyte having a pH between about 3.8 and about 4.6 comprising between about 40 to about 60 g. p. l. of nickel, about 18 to about 30 g. p. l. of sodium, about 27 to about 51 g. p. l. of chloride radical, about 65 to about 99 g. p. l. of sulfate radical, about 15 to about 25 g. p. l. of boric acid and about 0.0004 to about 0.0008 g. p. l. of a compound having the structural formula



with the balance essentially water, and electrolyzing said catholyte while maintaining the temperature between about 130° F. and about 150° F. by passing electric current at a current density between about 12 and about 25 amperes per square foot through said electrolyte from an anode to a cathode to deposit sound nickel cathodes.

9. A nickel electrorefining electrolyte having a pH between about 3 and about 5 and containing about 40 to about 70 g. p. l. of nickel, about 12 to about 30 g. p. l. of sodium, about 18 to about 55 g. p. l. of chloride radical, about 65 to about 115 g. p. l. of sulfate radical, about 15 to about 25 g. p. l. of boric acid and about 0.0003 to about 0.001 g. p. l. of at least one terminally substituted polyethylene oxide condensate selected from the group consisting of a polyethylene oxide condensate of m-methyl p-octyl phenol containing 8 to 11 moles of ethylene oxide per mole and a polyethylene oxide condensate of lauryl alcohol containing 4 to 6 moles of ethylene oxide per mole, the balance being essentially water.

10. A nickel electrorefining electrolyte having a pH between about 3 and about 5 and contain-

ing about 40 to about 70 g. p. l. of nickel, about 12 to about 30 g. p. l. of sodium, about 18 to about 55 g. p. l. of chloride radical, about 65 to about 115 g. p. l. of sulfate radical, about 15 to about 25 g. p. l. of boric acid and about 0.0003 to about 0.001 g. p. l. of a compound having the structural formula



where  $m$  is 8 to 11

the balance being essentially water.

11. A nickel electrorefining electrolyte having a pH between about 3 and about 5 and containing about 40 to about 70 g. p. l. of nickel, about 12 to about 30 g. p. l. of sodium, about 18 to about 55 g. p. l. of chloride radical, about 65 to about 115 g. p. l. of sulfate radical, about 15 to about 25 g. p. l. of boric acid and about 0.0003 to about 0.001 g. p. l. of a compound having the structural formula



the balance being essentially water.

12. A nickel electrorefining electrolyte having a pH between about 3 and about 5 and containing about 40 to about 70 g. p. l. of nickel, about 12 to about 30 g. p. l. of sodium, about 18 to about 55 g. p. l. of chloride radical, about 65 to about 115 g. p. l. of sulfate radical, about 15 to about 25 g. p. l. of boric acid and about 0.0003 to about 0.001 g. p. l. of a compound having the structural formula



the balance being essentially water.

13. A nickel electrorefining electrolyte having a pH between about 3.8 and about 4.6 and containing about 40 to about 60 g. p. l. of nickel, about 18 to about 30 g. p. l. of sodium, about 27 to about 51 g. p. l. of chloride radical, about 65 to about 99 g. p. l. of sulfate radical, about 15 to about 25 g. p. l. of boric acid and about 0.0004 to about 0.0008 g. p. l. of at least one terminally substituted polyethylene oxide condensate selected from the group consisting of a polyethylene oxide condensate of m-methyl p-octyl phenol containing 8 to 11 moles of ethylene oxide per mole and a polyethylene oxide condensate of lauryl alcohol containing 4 to 6 moles of ethylene oxide per mole, the balance being essentially water.

14. A nickel electrorefining electrolyte having a pH between about 3.8 and about 4.6 and containing about 40 to about 60 g. p. l. of nickel, about 18 to about 30 g. p. l. of sodium, about 27 to about 51 g. p. l. of chloride radical, about 65 to about 99 g. p. l. of sulfate radical, about 15 to about 25 g. p. l. of boric acid and about 0.0004 to about 0.0008 g. p. l. of a compound having the structural formula



where  $m$  is 8 to 11

the balance being essentially water.

15. A nickel electrorefining electrolyte having a pH between about 3.8 and about 4.6 and containing about 40 to about 60 g. p. l. of nickel, about 18 to about 30 g. p. l. of sodium, about 27 to about 51 g. p. l. of chloride radical, about 65 to about 99 g. p. l. of sulfate radical, about

## 11

15 to about 25 g. p. l. of boric acid and about 0.0004 to about 0.0008 g. p. l. of a compound having the structural formula



the balance being essentially water.

16. A nickel electrorefining electrolyte having a pH between about 3.8 and about 4.6 and containing about 40 to about 60 g. p. l. of nickel, about 18 to about 30 g. p. l. of sodium, about 27 to about 51 g. p. l. of chloride radical, about 65 to about 99 g. p. l. of sulfate radical, about 15 to about 25 g. p. l. of boric acid and about

## 12

0.0004 to about 0.0008 g. p. l. of a compound having the structural formula



5 the balance being essentially water.

## References Cited in the file of this patent

## UNITED STATES PATENTS

| 10 | Number    | Name             | Date          |
|----|-----------|------------------|---------------|
|    | 1,970,578 | Schoeller et al. | Aug. 21, 1934 |
|    | 2,294,311 | Lind             | Aug. 25, 1942 |
|    | 2,480,771 | Renzoni          | Aug. 30, 1949 |